

March 3, 1936.

F. F. CRAMER ET AL

2,032,738

MAKING OF RAILROAD RAILS

Filed May 21, 1934

2 Sheets-Sheet 1



*Fig. 2.*



*Inventors:*

FRANK F. CRAMER and  
HARRY H. LOCKE.

*by:*

*Usina & Rauber*  
Their Attorneys.

March 3, 1936.

F. F. CRAMER ET AL

2,032,738

MAKING OF RAILROAD RAILS

Filed May 21, 1934

2 Sheets-Sheet 2

*Fig. 3.*



*Fig. 4.*



*Inventors:*

FRANK F. CRAMER and  
HARRY H. LOCKE.

*By: Usina Rubber  
Their Attorneys*

## UNITED STATES PATENT OFFICE

2,032,738

## MAKING OF RAILROAD RAILS

Frank F. Cramer, Swissvale, and Harry H. Locke,  
Wilkinsburg, Pa.

Application May 21, 1934, Serial No. 726,784

## 1 Claim. (Cl. 148—21)

This invention relates to the making of railroad rails, one of the objects being to produce rails whose ends are more resistant to the pounding action of the wheels of passing traffic. Other 5 objects may be inferred.

Referring to the accompanying drawings:

Figure 1 is a plan of a rolling mill arrangement showing the features of the present invention.

Figure 2 is an elevation of the end of a rail- 10 road rail produced by the above arrangement.

Figure 3 is an enlargement from Figure 1.

Figure 4 is a cross-section of Figure 3.

These drawings show the finishing train 1 of a rail mill with a delivery table 2 leading away from 15 it past four hot-saws 3, the latter being mounted on the free ends of tilting arms 4 and being connected by belts 5 to individual motors 6. An operator's pulpit 7 is opposite these saws and is provided with the various controls necessary for 20 their operation. The table 2 terminates beyond the saws at a point where it may deliver rails to a second conveyer 8 which serves cooling beds 9. The arrangement is conventional as so far de- 25 scribed.

25 Rail-sectioned pieces leave the train 1 at temperatures slightly above the upper critical range of the steel from which they are rolled. They are of such lengths that two or three suitably lengthed rails may be cut from each by the hot-saws 3. The resulting rails are then delivered to the conveyer 8 from which they are laterally dragged to the cooling beds 9. The hot-saws 3 are arranged to simultaneously cut the pieces and are as close to the finishing train 1 as is mechani- 30 cally possible. Therefore, the pieces which have just left the train 1 are still above their upper critical range during this sawing and for a short time thereafter. They generally cool below this range as they are being dragged from the conveyer 8 or very shortly after they are on the cool- 35 ing beds 9. It is to be understood that they were originally in the form of ingots or blooms.

According to the present invention, spray-heads 40 10 are arranged adjacent the saws 3 so as to spray the opposite ends of the tops of the heads of rails 45 while they are on the table 2 in cutting positions respecting these saws. These spray-heads are all connected to a pipe line 11 by hoses 12, and this pipe line is supplied with a quenching fluid by a 50 pipe 13 through an electrically operated valve 14. The quenching fluid may be any medium which will quickly cool steel when brought into contact with it.

The valve 14 may be directly controlled through 55 a line 15 by a push-button 16 located in the oper-

ator's pulpit 7. If automatic operation is desired, it may be operated by a limit switch 17, which is associated with one of the arms 4, through lines 18 and an interposed electric timer 19. A power supply 20 powers both the lines 15 5 and 18. For convenience, all of the lines are illustrated by single lines on the drawings, but it should be understood that they may be commercial cables, each containing the required number of conductors. The electrically operated valve 14 10 and the timer 19 may be any of those commercially available.

Referring again to the spray-heads 10, it is to be observed that there is just one of these at each of the end saws and that there are two at the two 15 middle saws. In all cases, they are arranged so as to be opposite the ends of rails cut by the hot-saws 3. In mills using only three saws, the same relationship will be maintained, there being then only one double arrangement of the spray-heads 20 which will be at the center one of the saws.

The rail-sectioned pieces are ordinarily carried on their sides by the delivery table 2, the heads of these pieces being away from the center line of the saws. Each of the spray-heads 10 consists of a header 21 from which a series of nozzles 22 extend towards the heads of the pieces on the delivery table. These nozzles are arranged to parallel the end portions of the rails cut by the saws and are characterized in that they progressively decrease in size away from the one closest to the one of the saws that is adjacent that particular head.

The operation of the foregoing will now be described, it being understood that this operation 35 constitutes a new method of making railroad rails which may be likewise carried out by the use of other apparatus than that just described.

Ingots or blooms heated to proper rolling temperatures are rolled into rail-sectioned pieces by 40 the rail mill. These pieces leave the finishing train 1 and are carried by the delivery table 2 into proper cutting positions respecting the hot-saws 3. The operator in the pulpit 7 controls these operations and successively effects operation of 45 the saws 3 so as to cut the extreme ends of the pieces while simultaneously making two other cuts at spaced points so that suitably lengthed rails result. This is done as soon as possible after the hot-rolling operation, this meaning that the hot-saws must be as close as is possible to the finishing train.

The operator pushes the button 16 so as to apply the quenching medium to the end portions of the tops of the heads of the rails after the cutting 55

has started or immediately upon its completion. If the limit switch 17 is used, the arrangement should be such that the circuit to the timer 19 is closed at some time during the actual cutting of the pieces or immediately thereafter. The timer 19 is then set to cause quenching of the rail ends to cease after a certain interval of time. If the limit switch is set so that the quenching is done while the saws are still cutting, care must be taken that the rail heads do not begin hardening too soon, since otherwise the saws will be damaged.

In the case of the spray-heads illustrated, the application of the quenching medium will be proportioned so that the quenching is greatest at their extreme ends and gradually decreases away from the same. It is obvious that this quenching may be otherwise proportioned to produce the same effects. In all cases the application of the quenching fluid is proportioned so that the quenching effects extend only short distances beneath the tops of the heads of the rails, and is stopped while there is still sufficient heat left in the rails to draw the affected portions sufficiently to eliminate internal strains. In the case of the automatic arrangement illustrated, the electric timer 19 is set to stop the quenching at a proper time for this purpose. The rails are then delivered to the conveyor 8 and dragged to the cooling beds 9.

To aid in disclosing the above method, a rather specific example will now be disclosed. It may be assumed that the rails being rolled are of the ordinary weights now currently used by the railroads, and that the quenching fluid is water at temperatures ordinarily found in the pipe lines serving a rail mill. Immediately upon the completion of the cutting of the pieces into such rails by the hot-saws, the water is applied against the tops of their heads. With an arrangement similar to the one illustrated and described, the rails will still be above their upper critical ranges so that hardening will result. The application of the spray should be proportioned so that the hardening effect extends to a depth of about three-quarters of an inch beneath the tops of the heads of the rails, and extends a longitudinal distance of not more than ten inches. If the water is applied in reasonable amounts, the time period required should not be more than from

ten to twenty seconds in order to produce the results described.

So far as is known, the present inventors are the first to produce a railroad rail having a hardened end. A rail produced by their method and apparatus is characterized by having the top of its head hardened at at least one end to a depth of not more than .75 inch and to a longitudinal distance of not more than ten inches, the hardened area gradually decreasing in depth away from the extreme end of the rail and being practically free from internal strains. The gradual decrease in depth is obtained by the use of the spray-heads described, while the freedom of strain results from the discontinuance of the quenching at a time when there is still sufficient heat left in the rails to draw back the hardened area.

The gradual decrease in depth is of value because it prevents any tendency of the hardened area to shatter under the pounding impact of the wheels of traffic. Ordinarily, the effective hardened surface will not extend more than from six to eight inches away from the extreme end of the rail.

Figure 2 shows the general shape of the hardened area. It might be mentioned that a somewhat similar shape results even if the quenching is done evenly instead of in diminishing amounts, since the longitudinal heat transmission along the rail will effect this result.

We claim:

A method of making railroad rails, including hot-rolling ingots or blooms into rail-sectioned pieces, cutting said pieces into suitably lengthed rails as soon as possible after the completion of said hot-rolling, and applying a quenching medium to the end portions of the tops of the heads of said rails after said cutting has started or immediately upon its completion, the application of said quenching medium being proportioned so that the quenching effects extend only short distances beneath said tops and so that they are greatest at their extreme ends and gradually decrease away therefrom, said application being stopped while there is still sufficient heat left in said rails to draw the affected portions sufficiently to eliminate internal strains.

FRANK F. CRAMER.  
HARRY H. LOCKE.

50